

## 1

2,977,261

## HEAT-TREATMENT OF TITANIUM-COPPER ALLOYS

Marion Katherine McQuillan, Birmingham, and Jack Reynolds, Walsall, England, assignors to Imperial Chemical Industries Limited, London, England, a corporation of Great Britain

No Drawing. Filed Jan. 26, 1959, Ser. No. 788,793

Claims priority, application Great Britain Jan. 29, 1958

10 Claims. (Cl. 148—12.7)

This invention relates to a method of heat treating titanium alloys containing copper.

Alloys of titanium containing copper have been disclosed and it has also been proposed to heat treat such alloys by age-hardening methods. Various temperatures and periods of treatment produced only relatively small changes in hardness in a titanium-copper alloy. In addition such alloys have been reported to undergo overageing after comparatively short ageing times of the order of 2 hours.

The object of the present invention is to provide a method of heat treating titanium-copper alloys whereby improved properties are obtained.

According to the invention there is provided a method of treating a titanium-base alloy containing between 0.9% and 2.6% of copper, balance titanium apart from impurities, which comprises heating the alloy to a temperature between 750° C. and 1000° C. for a period of not less than 5 minutes and cooling the alloy at a rate sufficient to retain the alloy constituents in solid solution. Such a process is hereinafter referred to as "solution-treatment."

Alloys treated in accordance with this aspect of the invention have improved elevated temperature properties compared with similar alloys subjected to a preliminary annealing treatment at a temperature outside the above range.

By way of example, a titanium-2% copper alloy, solution-treated at 800° C. has, when tested at 220° C., an ultimate tensile strength of 27.5 tons/sq. in., a 0.1% proof stress of 19.8 tons/sq. in. and an elongation of 31%, whereas, a similar alloy solution-treated at 800° C. and then annealed for ½ hour at 655° C. has an ultimate tensile strength of 22.9 tons/sq. in., a 0.1% proof stress of 15.0 tons/sq. in. and an elongation of 23%.

According to a feature of the invention, the alloy, after cooling, is heated to a temperature between 300° C. and 600° C. for a period between 10 and 1000 hours.

Improvements in tensile properties and hardness associated with good ductility and good creep and fatigue properties are obtained by subjecting the alloy to both solution-treatment and ageing-treatment.

The preferred range of composition is 1.8 to 2.2% copper. The interstitial impurity content of the alloy may vary between wide limits without loss of age-hardenability. Taking the hardness of the titanium starting material as a measure of oxygen and nitrogen content, age-hardening has been observed between the limits 70 and 200 on the Vickers scale of hardness numerals, the preferred range being 120 to 160 Vickers Diamond Pyramid Hardness Numerals.

The heat treatment may be carried out in air or in a controlled atmosphere.

The alloys may be solution treated at any temperature between 750° C. and 1000° C., i.e. within the alpha, the beta or the alpha plus beta phase fields. Subsequent age-hardening is greatest when the microstructure of the solu-

## 2

tion-treated alloy consists essentially of equiaxed grains of the alpha phase, but the presence of a small quantity of the beta phase may be beneficial. The preferred range is therefore 780 to 810° C. The duration of the solution-treatment may be any period in excess of 5 minutes, preferably between 10 minutes and 1 hour. After solution-treatment the alloys may be water-quenched or air-cooled without significant change in the age-hardening characteristics.

10 Age-hardening may be carried out at any temperature between 300° C. and 600° C. but the preferred temperatures are those between 350° C. and 450° C. For any given ageing temperature, the hardness peak may be reached in times varying between ¼ hour and 1000 hours, but the preferred ageing time is 10 to 300 hours. Some improvement in hardness over that obtained by ageing for the preferred time may be brought about by ageing for prolonged periods of up to 1000 hours. At the end of the ageing treatment, the alloys may be water-quenched or air-cooled, i.e. allowed to cool at a natural rate in air. Annealing to soften the material, intermediate between rolling passes, may be carried out in the range 650° C. to 750° C. for periods of ½ hour to 2 hours. Solution-treatment and ageing may afterwards be carried out. In Table 25 I are given details of various treatments in accordance with the invention and the effects of varying different factors such as composition, temperature and times. Except where indicated in the first column of this table, the titanium raw material used to make the alloys was within 30 the preferred range of hardness (120 to 160 Vickers D.P.N.).

The ultimate tensile strength, proof stress and ductility in the solution-treated condition indicate that the alloys can be rolled easily in that condition. On ageing, increases in proof stress and ultimate tensile strength occur corresponding to the increase in hardness.

Table II shows the tensile properties of a titanium-2% copper alloy solution-treated in the alpha-phase field and aged for 238 hours at 400° C. It will be observed that, on ageing, there is an increase in strength without significant loss of ductility.

Whilst improved properties are conferred upon the alloy by the solution-treatment and ageing procedure discussed above, a reduction of the ageing period is produced by cold working the alloy after the solution-treatment. Reductions of between 2 and 25% accelerate ageing so that the preferred ageing period is decreased by a factor of between 2 and 4. It has been found that after solution-treatment and cold working to effect 10% reduction, an ageing period of 20 to 60 hours is required to produce similar properties to those possessed by the alloy after solution-treating and ageing for 160 to 320 hours but without cold working.

## 55 EXAMPLE 1

A titanium-2% copper alloy is heated to a temperature of 800° C. for a period of 30 minutes and air cooled. The alloy is then reduced 10% by cold rolling and aged at 400° C. for 46 hours. After solution-treatment the Diamond Pyramid Hardness Numeral is 185, after cold rolling 233, and after ageing 272.

For comparison with the foregoing example, a hardness of 259 is obtained when a similar alloy is solution-treated as in the example and aged for 140 hours, but not cold worked after solution-treatment. Thus, in this example, the ageing time is reduced by a factor of approximately 3 when the cold rolling step is added in accordance with the invention.

70 The invention is applicable to the manufacture of a variety of products and articles formed from the titanium-base alloy herein referred to, such as rod, forgings and, in particular, sheet. It is advantageous in the case of

sheet, to cold roll and fabricate after solution-treatment and then to develop the improved properties subsequently by ageing.

8. A method of treating a titanium-base alloy consisting of between 1.8 and 2.2% copper, balance titanium apart from impurities, which comprises heating the alloy

Table I

| Composition<br>(inc. quality<br>of titanium) | Softening Anneal |              |                   | Solution Treatment |             |                   | Ageing Treatment |              |                   | Hardness<br>(D.P.N.) | Hard-<br>ness In-<br>crement<br>(per-<br>cent) | Illustrative of— |
|----------------------------------------------|------------------|--------------|-------------------|--------------------|-------------|-------------------|------------------|--------------|-------------------|----------------------|------------------------------------------------|------------------|
|                                              | Temp.,<br>° C.   | Time,<br>hr. | Terminated<br>by— | Temp.,<br>° C.     | Time        | Terminated<br>by— | Temp.,<br>° C.   | Time,<br>hr. | Terminated<br>by— |                      |                                                |                  |
| 1.5% Cu                                      |                  |              |                   | 800                | 1 hr.....   | Quench            | 400              | 224          | Quench.....       | 185                  | 224                                            | 21               |
| 2.3% Cu                                      |                  |              |                   | 800                | 1 hr.....   | do.....           | 400              | 224          | do.....           | 255                  | 280                                            | 10               |
| 2.0% Cu                                      |                  |              |                   | 800                | 1 hr.....   | do.....           | 400              | 224          | do.....           | 203                  | 264                                            | 31               |
| 2.0% Cu-71<br>D.P.N.<br>titanium.            |                  |              |                   | 800                | 1 hr.....   | do.....           | 400              | 230          | do.....           | 128                  | 223                                            | 74               |
| 2.0% Cu                                      |                  |              |                   | 1,000              | 1/4 hr..... | do.....           | 400              | 230          | do.....           | 253                  | 288                                            | 12               |
| 2.0% Cu                                      | 700              | 1            | Air cool...       | 800                | 10 min..... | do.....           | 400              | 238          | do.....           | 195                  | 280                                            | 41               |
| 2.0% Cu                                      |                  |              |                   | 800                | 1 hr.....   | Air cool...       | 400              | 238          | Air cool...       | 203                  | 275                                            | 35               |
| 2.0% Cu                                      |                  |              |                   | 800                | 1 hr.....   | Quench            | 400              | 730          | Quench...         | 203                  | 275                                            | 35               |

Table II

| Condition of Alloy    | Hardness<br>(D.P.N.) | U.T.S.<br>(ton/sq. in.) | Tensometer<br>Yield Pt.<br>(ton/sq. in.) | Elongation<br>(percent on<br>4 $\sqrt{A}$ ) | Percent Re-<br>duction in<br>Area | Percent In-<br>crease in<br>U.T.S. on<br>ageing |
|-----------------------|----------------------|-------------------------|------------------------------------------|---------------------------------------------|-----------------------------------|-------------------------------------------------|
| Solution-treated..... | 186                  | 38.2                    | 30.2                                     | 29                                          | 50-55                             | —                                               |
| Aged.....             | 265                  | 52.9                    | 45.6                                     | 24                                          | 36                                | 38                                              |

We claim:

1. A method of treating a titanium-base alloy consisting of between 0.9% and 2.6% copper, balance titanium apart from impurities, which comprises heating the alloy to a temperature between 750° C. and 1000° C. for a period of not less than 5 minutes and cooling the alloy at a rate sufficient to retain the alloy constituents in solid solution, cold-working the alloy to effect a reduction of between 2% and 25%, and heating the alloy to a temperature between 300° C. and 600° C. for a period between 10 and 1000 hours.

2. A titanium-base alloy produced by the method of claim 1.

3. A method of treating a titanium-base alloy consisting of between 1.8% and 2.2% copper, balance titanium apart from impurities, which comprises heating the alloy to a temperature between 780° C. and 810° C. for a period between 10 minutes and 1 hour, cooling the alloy in air substantially to room temperature, cold-rolling the alloy to effect a reduction of between 2% and 25%, and heating the alloy to a temperature between 350° C. and 450° C. for a period between 10 and 300 hours.

4. A titanium-base alloy produced by the method of claim 3.

5. A method of treating a titanium-base alloy consisting of between 0.9% and 2.6% copper, balance titanium apart from impurities, which comprises heating the alloy at a temperature between 750° C. and 1000° C. for a period of not less than 5 minutes, cooling the alloy at a rate sufficient to retain the alloy constituents in solid solution and age-hardening the alloy by heating at a temperature between 300° C. and 600° C. for a period between 20 and 1000 hours.

6. A titanium-base alloy produced by the method of claim 5.

7. A method of treating a titanium-base alloy as set forth in claim 5 in which the age-hardening heat-treatment is carried out for about 160 to 320 hours.

40 to a temperature between 780° C. and 810° C. for a period between 10 minutes and 1 hour, cooling the alloy in air substantially to room temperature, and heating the alloy to a temperature between 350° C. and 450° C. for a period between 20 and 300 hours.

45 9. A titanium-base alloy produced by the method of claim 8.

50 10. A method of treating a titanium-base alloy consisting of between 1.8 and 2.2% copper, balance titanium apart from impurities which comprises heating the alloy to a temperature between 780° C. and 810° C. for a period between 10 minutes and 1 hour, cooling the alloy in air substantially to room temperature, and heating the alloy to a temperature between 350° C. and 450° C. for a period between 160 and 320 hours.

#### References Cited in the file of this patent

#### UNITED STATES PATENTS

2,797,996 Jaffee et al. \_\_\_\_\_ July 2, 1957  
2,857,269 Vordahl \_\_\_\_\_ Oct. 21, 1958

#### OTHER REFERENCES

Titanium Project PB 103370, The Manufacture of Ductile Ti and Ti Alloys, Report No. 17; period covered Apr. 1, 1947 to Sept. 1, 1948; page 35; released June 15, 1951.

65 Handbook on Titanium, H. K. Adenstedt, August 1954; Wright Air Development Center, WADC Technical Report 54-305, part 1, pages II-2-1 and II-2-2, II-3-1 to II-3-19.

70 Hansen: Constitution of Binary Alloys, McGraw-Hill, pages 642-646, 1958.

Titanium, McQuillan and McQuillan, pages 362-363, 372-378, 1956.

Physical Metallurgy and Heat Treatment of Titanium Alloys, Mallory Sharon Ti Corp., pages 11-25, 1955.

75 The Iron Age, pages 162-168, Apr. 2, 1953.